

# UNITED STATES PATENT OFFICE.

ROBERT ATHELSTAN MARR, OF NORFOLK, VIRGINIA, ASSIGNOR TO GENERAL WATER-PROOFING CO., INCORPORATED, OF NORFOLK, VIRGINIA, A CORPORATION OF VIRGINIA.

## PROCESS OF WATERPROOFING TEXTILE MATERIAL AND PRODUCT THEREOF.

1,121,648.

Specification of Letters Patent. Patented Dec. 22, 1914.

No Drawing.

Application filed January 13, 1914. Serial No. 811,912.

*To all whom it may concern:*

Be it known that I, ROBERT ATHELSTAN MARR, a citizen of the United States, residing at Norfolk, in the county of Norfolk and State of Virginia, have invented certain new and useful Improvements in Processes of Waterproofing Textile Material and Products Thereof, of which the following is a specification.

10 The present invention relates to the treatment of materials composed of textile fibers, such as fabrics, rope, yarn and the like, by impregnating the same with a treating medium containing paraffin, rosin and diatomaceous earth.

15 The invention includes the treatment of all materials composed of textile fibers such as duck, canvas, rope, cordage, nets for fishing, hammocks, bags and bagging, and I 20 desire to call attention to the fact that these materials may be treated either in the finished form, or in the form of the yarn or small string, from which the materials are to be made.

25 In carrying out my process the bath employed may consist of paraffin, 100 parts; diatomaceous earth, 2 to 10 parts; and rosin 3 to 10 parts; to which Paris green 1 to 2 parts, and any dye soluble in the menstrum, 30 in suitable quantity may be added if desired, for giving special effects, the addition of these last two being optional. The proportions may also be varied, to suit particular conditions.

35 The material to be treated may be in the air-dry condition, containing 5 to 15% of moisture, although for securing heavy impregnation it is advisable sometimes to use material containing more moisture than 40 this.

45 I call attention to the fact that rope and other materials treated with the mixture herein described becomes stronger than such rope or similar material before treatment, thereby producing a material advantage over the use of tar for impregnating such materials, since tar weakens the rope and other materials, and some varieties of tar appear to act injuriously on the textile

50 fibers, possibly on account of the corrosive tar acids or other corrosive materials contained therein.

A further advantage in the use of this

mixture consists in that the rope or other material when so treated will float, although 55 its weight has been somewhat increased, but the exclusion of the water by the impregnated material which I employ prevents the rope from absorbing water, and thereby becoming heavy enough to sink. This is a 60 material advantage in ropes used for towing lines, casting lines, and the like.

The materials when treated according to this process are preserved against the action of dry rot, marine insects, (teredo, 65 limnoria, barnacles, etc.) fish slime, and the like, all of which cause the materials mentioned to deteriorate very rapidly. The material is rendered impervious to water, acids 70 and the like.

The material being treated may be submerged in the bath, while said bath is maintained at a temperature of somewhat above the boiling point of water, say 230 to 250° F., and the bath may be allowed to cool 75 almost down to the solidifying point of bath if a heavy impregnation is desired, or may be allowed to cool only a few degrees, if a light impregnation is desired.

By the use of the oil soluble dye I can 80 produce any desired color, in the material treated, which will not wash out, and in most instances, will not fade away when exposed to the action of sea water, sunlight, and other conditions under which colors 85 ordinarily fade more or less.

I call particular attention to the use of this process in the treatment of bags for holding cement, fertilizer, and various other materials, or the fabric from which said 90 bags are to be made. The light impregnation of the fabric or other material may be produced by treating fabric which is in its air dry condition, while the use of fabric or the like containing more moisture than this 95 leads to a heavier impregnation suitable for other purposes. The material may be soaked in water, prior to the immersion in the bath, if desired. This process also finds special application in the treatment of canvas or duck for life preservers, tents, sails, etc.

By regulating the amount of the preservative, impermeabilizing solution, I can produce products which are quite stiff, or very 105 flexible.

I desire to call attention to the absence of volatile solvents from the treating bath, since the evaporation of these solvents, heretofore proposed in impregnating materials of this character, leaves the material more or less porous, and carries the treating agent to the surface of the fabric, etc., under treatment, leaving less of the impregnating or filling agent in the inner parts of the materials.

10 The use of rosin in the bath renders the process especially valuable in the manufacture of belting since it acts to prevent the slipping of belts on the pulleys. The rosin aids the impregnation of the textile material with the constituents of the bath.

20 Materials comprising both fabric and rope, *e. g.* reinforced belts, tents and the like may be treated by this process, and in the case of stitched articles, bags, etc., the thread is treated as well as the fabric, either before or after the stitching operation.

25 The use of Paris green is especially recommended in treating fish nets, ropes which are kept for long periods in salt water, balloon bags, and the like.

30 While the diatomaceous earth is an extremely finely divided material, and will permeate the pores of the individual fibers, the Paris green is much coarser and does not penetrate so deeply, but remains as a coating, on or near the surface.

35 The impregnation of textile materials with a mixture including diatomaceous earth, paraffin and naphthalene, with or without rosin and Paris green, is described and claimed in my copending application Serial No. 811,911, filed concurrently herewith.

40 The treatment of fabrics forming portions of life preservers is also covered by my applications Serial Nos. 811,909 and 811,910, filed concurrently herewith.

What I claim is:

45 1. A process of treating materials composed of textile fibers which comprises impregnating the same with a preservative, waterproofing, impermeabilizing agent, comprising diatomaceous earth, and a water-insoluble fluent carrier comprising a hydrocarbon body liquid at a temperature of 212° F., and rosin.

55 2. A process of treating materials composed of textile fibers which comprises impregnating the same with a preservative, water-proofing, impermeabilizing agent, comprising diatomaceous earth, and a water-insoluble fluent carrier comprising paraffin and rosin.

60 3. A process of treating materials composed of textile fibers which comprises impregnating the same with a preservative waterproofing, impermeabilizing agent, comprising diatomaceous earth, and a water-insoluble fluent carrier comprising a hydro-

carbon body existing as a liquid at temperatures near 212° F., a dye soluble therein, and rosin.

4. A process of treating cordage and fabrics, which comprises impregnating the same with a material including paraffin and diatomaceous earth, at a temperature above 212° F.

5. A process of treating cordage and fabrics, which comprises impregnating the same with a material including paraffin and diatomaceous earth, at a temperature above 212° F., and decreasing the temperature of the impregnating material during the process.

6. A process which comprises immersing articles composed essentially of textile fibers, in a bath comprising diatomaceous earth, paraffin and rosin, at a temperature above 212° F., and thereafter subjecting said materials to a bath containing molten paraffin, said bath having a lower temperature than that employed in said first step.

7. A process which comprises immersing articles composed essentially of textile fibers, in a bath comprising diatomaceous earth, paraffin and rosin, and a dye soluble in said mixture, at a temperature above 212° F., and thereafter subjecting said materials to a bath containing molten paraffin, said bath having a lower temperature than that employed in said first step.

8. A process which comprises impregnating textile materials with a mixture including a non-reactive impermeabilizing agent, liquid at temperatures near 212° F., and rosin, and a finely divided silicious material carried thereby.

9. Fabric and cordage impregnated with paraffin, diatomaceous earth and rosin.

10. Fabric and cordage impregnated with paraffin, a dye soluble therein, diatomaceous earth, and rosin.

11. A textile material impregnated with a preservative substance comprising a resolidified, non-reactive, impermeabilizing agent, liquid at temperatures above 212° F., a finely divided silicious material carried by said agent, and rosin.

12. A textile material impregnated with a preservative substance comprising a resolidified, non-reactive, impermeabilizing agent, liquid at temperatures above 212° F., a finely divided silicious material carried by said agent, and rosin, said material carrying a coating of a poisonous solid material.

13. A textile material impregnated with a preservative substance comprising a resolidified, non-reactive, impermeabilizing agent, liquid at temperatures above 212° F., a finely divided silicious material carried by said agent, and rosin, said material having a coating including Paris green.

14. A unitary article comprising in its structure, both fabric and cordage, said fabric and said cordage, being impregnated

with a preservative substance, comprising a resolidified, non-reactive, impermeabilizing agent, liquid at temperatures above 212° F., and solid at ordinary temperature, said impermeabilizing agent carrying a finely divided silicious material, and rosin.

In testimony whereof I have affixed my signature in presence of two witnesses.

ROBERT ATHELSTAN MARR.

Witnesses:

A. B. FOSTER,  
JANEY HOPE MARR.